

## 1

3,160,591

LUBRICATING OIL THICKENED TO A GREASE  
WITH A 1,3,5-TRIAZINE COMPOUNDRobert E. Halter, Verona, Paul R. McCarthy, Allison Park, and Joseph J. McGrath, Monroeville, Pa., assignors to Gulf Research & Development Company, Pittsburgh, Pa., a corporation of Delaware  
No Drawing. Filed Mar. 8, 1962, Ser. No. 178,285  
12 Claims. (Cl. 252—47)

This invention relates to an improved lubricating composition and more particularly to a lubricant suitable for high temperature lubrication.

The trend in design of modern aircraft has accentuated the need for greases which will lubricate anti-friction bearings operating at high rotational speeds and high temperatures. Considerable progress has been made in recent years in producing improved aircraft greases. For example, a number of greases are now available for lubricating bearings operating at 10,000 to 20,000 revolutions per minute at temperatures up to about 400° F. However, great difficulty has been encountered in producing a grease which will effectively lubricate bearings operating at speeds of 10,000 to 20,000 and more revolutions per minute and temperatures of about 400° to about 600° F. for prolonged periods of time.

We have discovered that a lubricating composition having improved lubricating characteristics for an extended period of time when used to lubricate bearings operating at temperatures up to about 600° F. and speeds of 10,000 to 20,000 and more revolutions per minute can be obtained by incorporating into a lubricating oil in oil thickening proportions a symmetrical triazine, i.e., a 1,3,5-triazine compound melting above about 400° F. (205° C.) having the following formula:



wherein R and R<sub>1</sub> are selected from the group consisting of hydrogen, alkyl, aryl, alkaryl, aralkyl, cyanoalkyl, pyridyl, amino, hydroxy and mercapto radicals, R and R<sub>1</sub> being unlike radicals when selected from the group consisting of amino, hydroxy and mercapto radicals. Thus, the improved lubricating composition of the present invention consists of a dispersion in a lubricating oil of a sufficient amount to thicken the lubricating oil to a grease consistency of a 1,3,5-triazine compound melting above about 205° C. of the type designated by the above structural formula. The lubricating composition of the invention can contain one or more of the triazine compounds. Especially preferred compositions consist of a lubricating oil thickened to the consistency of a grease with ammeline or ammelide or a mixture of ammeline and ammelide. When a mixture of ammeline and ammelide is employed, the weight ratio of the ammeline to ammelide is preferably about 1:1.

It will be noted that R and R<sub>1</sub> in the structural formula set forth hereinabove can be the same or different radicals when selected from the group consisting of hydrogen, alkyl, aryl, alkaryl, aralkyl, cyanoalkyl and

## 2

pyridyl radicals provided, of course, that the melting point of the compound is at least 205° C. When R and R<sub>1</sub> are selected from the group consisting of amino, hydroxy and mercapto radicals, the radicals should not all be the same. For example, we do not intend to include compounds such as cyanuric acid (s-triazinetriol) or melamine (2,4,6-triamino-s-triazine).

It should be understood that the symmetrical (s) triazine compounds can contain other substituents provided, of course, that said other substituents do not adversely affect the beneficial oil thickening properties of the s-triazine compounds.

An especially preferred group of triazine compounds for the purpose of the invention includes those compounds wherein each of the R radicals is either a hydroxy radical or an amino radical. When each of the R radicals is an amino radical, the resulting compounds are designated as guanamine derivatives. Preferred guanamine derivatives are those wherein R<sub>1</sub> is selected from the group consisting of hydrogen, alkyl (e.g., methyl, ethyl, propyl and n-butyl), aryl (e.g., phenyl and naphthyl), alkaryl (e.g., tolyl), aralkyl (e.g., benzyl), cyanoalkyl (e.g., cyanoethyl, cyanobutyl and cyanoctyl), pyridyl, hydroxy and mercapto radicals. When R<sub>1</sub> in the guanamine derivatives is an alkyl radical, it preferably is selected from the group consisting of methyl, ethyl, propyl and n-butyl radicals in order to give a compound having a melting point above about 205° C. When R<sub>1</sub> is isobutyl or a higher alkyl radical the melting point of the resulting substituted guanamine is below 205° C. While compounds melting below 205° C. can be used to produce grease compositions for use at temperatures below 400° F., such compounds are not satisfactory thickening agents for grease compositions used to lubricate bearings operating at high rotational speeds at temperatures of 400° to 600° F. and higher for prolonged periods of time. When R<sub>1</sub> in the guanamine derivatives is an alkaryl or an aralkyl radical, the alkyl portion of the alkaryl and aralkyl radicals preferably contains not more than 2 carbon atoms. When R<sub>1</sub> in the preferred guanamine derivatives is a cyanoalkyl radical, the alkyl portion of the cyanoalkyl radical can contain as many as 8 carbon atoms and still give a compound melting above 205° C.

Illustrative of the preferred guanamine derivatives which can be used in the present invention are the following:

- 2,4-diamino-1,3,5-triazine
- 2,4-diamino-6-methyl-1,3,5-triazine
- 2,4-diamino-6-ethyl-1,3,5-triazine
- 2,4-diamino-6-propyl-1,3,5-triazine
- 2,4-diamino-6-n-butyl-1,3,5-triazine
- 2,4-diamino-6-phenyl-1,3,5-triazine
- 2,4-diamino-6- $\alpha$ -naphthyl-1,3,5-triazine
- 2,4-diamino-6- $\beta$ -naphthyl-1,3,5-triazine
- 2,4-diamino-6-m-tolyl-1,3,5-triazine
- 2,4-diamino-6-p-tolyl-1,3,5-triazine
- 2,4-diamino-6-benzyl-1,3,5-triazine
- 2,4-diamino-6-cyanoethyl-1,3,5-triazine
- 2,4-diamino-6-cyanobutyl-1,3,5-triazine
- 2,4-diamino-6-cyanoctyl-1,3,5-triazine
- 2,4-diamino-6-pyridyl-1,3,5-triazine
- 2,4-diamino-6-hydroxy-1,3,5-triazine
- 2,4-diamino-6-mercaptop-1,3,5-triazine

While the guanamine derivatives of the above type are all effective thickeners for the preparation of high temperature greases, it is not to be implied that all serve with equal efficiency, since the various compounds may vary to some extent depending upon the nature and severity of the service to which they are subjected. That guanamine derivative which contains a hydroxy radical, i.e., 2,4-diamino-6-hydroxy-1,3,5-triazine (ammeline) is an especially preferred compound for use in the grease composition of the present invention.

The 1,3,5-triazine compounds can be prepared according to known chemical procedures. Neither the compounds per se nor their preparation constitutes any portion of the invention. For example, a 2-amino-4,6-dialkyl-1,3,5-triazine can be prepared by reacting a nitrile with guanidine. A 2,6-diamino-4-alkyl-1,3,5-triazine can be prepared by reacting alkyl biguanides with acylating agents in the presence of alkali. Acetoguanamine (2,4-diamino-6-methyl-1,3,5-triazine) having a melting point of 271° to 273° C. can be prepared by reacting dicyandiamide and acetonitrile in the presence of piperidine. Benzoguanamine (2,4-diamino-6-phenyl-1,3,5-triazine) having a melting point of 222° C. can be prepared by reacting dicyandiamide and benzonitrile in the presence of piperidine. 2,4-diamino-6-(2'-naphthyl)-1,3,5-triazine having a melting point of 240° C. can be prepared by reacting beta-naphthonitrile and dicyandiamide in the presence of piperidine. 2,4-diamino-6-benzyl-1,3,5-triazine having a melting point of 232° C. can be prepared by reacting dicyandiamide and benzylcyanide in the presence of piperidine. The preparation of some of the 1,3,5-triazines is more fully described in U.S. Patent No. 2,527,314, issued October 24, 1950 to Johnstone S. Mackay; U.S. Patent No. 2,302,162, issued November 17, 1942, to Werner Zerweck et al.; and U.S. Patent No. 2,408,694, issued October 1, 1946 to John Kenson et al.

The amount of the 1,3,5-triazine compound which we use is an amount sufficient to thicken the lubricating oil to a grease consistency. The exact amount in terms of weight percent may vary over wide limits depending upon the particular oil with which the triazine compound is to be blended and upon the properties desired in the final lubrication composition. While as much as 45 percent by weight of the total composition may comprise the triazine compound, we prefer to use smaller amounts, that is, in the order of about 20 to about 40 percent by weight. It should be understood, however, that, depending upon the consistency of the composition desired less than 20 percent or more than 45 percent of the triazine compound may be employed. In general, however, the 1,3,5-triazine compound comprises about 20 to about 45 percent by weight of the total composition.

The lubricating oil in which the triazine compound is incorporated is preferably a lubricant of the type best suited for the particular use for which the ultimate composition is designed. Since many of the properties possessed by the lubricating oil are imparted to the ultimate lubricating composition, we advantageously employ an oil which is thermally stable at the contemplated lubricating temperature. Some mineral oils, especially hydrotreated mineral oils, are sufficiently stable to provide a lubricating base for preparing lubricants to be used under moderately elevated temperatures. In general, however, where temperatures in the order of 400° to 600° F. are encountered, synthetic oils form a preferred class of lubricating bases because of their high thermal stability. The synthetic oil can be an organic ester which has a majority of the properties of a hydrocarbon oil of lubricating grade such as di-2-ethylhexyl sebacate, dioctyl phthalate and dioctyl azelate. Instead of an organic ester, we can use polymerized olefins, copolymers of alkylene glycols and alkylene oxides, polyorgano siloxanes, polyaryl ethers and the like.

The liquid polyorgano siloxanes and certain polyaryl

ethers because of their exceedingly high thermal stability form a preferred group of synthetic oils to which the triazine compound is added. The polyorgano siloxanes are known commercially as silicones and are made up of silicon and oxygen atoms wherein the silicon atoms may be substituted with alkyl, aryl, alkaryl, aralkyl and cycloalkyl radicals. Exemplary of such compounds are the dimethyl silicone polymers, diethyl silicone polymers, ethyl-phenyl silicone polymers and methyl-phenyl silicone polymers. Exemplary of the polyaryl ethers are the polyphenyl ethers, i.e., m-bis(m-phenoxyphenoxy) benzene and m-bis(m-phenoxyphenoxy) phenyl ether.

If desired, a blend of oils of suitable viscosity may be employed as the lubricating oil base instead of a single oil by means of which any desired viscosity may be secured. Therefore, depending upon the particular use for which the ultimate composition is designed, the lubricating oil base may be a mineral oil, a synthetic oil, or a mixture of mineral and/or synthetic oils. The lubricating oil content of the compositions prepared according to this invention comprises about 55 to about 80 percent by weight of the total composition.

In compounding the compositions of the present invention, various mixing and blending procedures may be used. In a preferred embodiment of the invention, the lubricating oil and the triazine compound together with conventional lubricant additives, if desired, are mixed together at room temperature for a period of about 10 to 30 minutes to form a slurry. During this initial mixing period some thickening is evidenced. Some lumps may be formed. The slurry thus formed is then subjected to a conventional milling operation in a ball mill, a colloid mill, homogenizer or similar device used in compounding greases to give the desired degree of dispersion. In the illustrative compositions of this invention, the slurry was passed twice, by means of a pump, through a Premier Colloid Mill set at a stator-rotor clearance of 0.002 inch. Maximum thickening occurred on the second pass through the mill.

The lubricating composition of this invention can contain conventional lubricant additives, if desired, to improve other specific properties of the lubricant without departing from the scope of the invention. Thus, the lubricating composition can contain a filler, a corrosion and rust inhibitor, an extreme pressure agent, an antioxidant, a metal deactivator, a dye and the like. Whether or not such additives are employed and the amounts thereof depend to a large extent upon the severity of the conditions to which the composition is subjected and upon the stability of the lubricating oil base in the first instance. Since the polyorgano siloxanes, for example, are in general more stable than mineral oils, they require the addition of very little, if any, oxidation inhibitor. When such conventional additives are used they are generally added in amounts between about 0.01 and 5 percent by weight based on the weight of the total composition.

In order to illustrate the lubricating characteristics of grease compositions of the invention when used to lubricate bearings operating at 400° to 600° F. and at rotational speeds of 10,000 to 20,000 and more revolutions per minute, a slight modification of the test procedure outlined by the Coordinating Research Council Tentative Draft (July 1954), "Research Technique for the Determination of Performance Characteristics of Lubricating Grease in Antifriction Bearings at Elevated Temperatures," CRC Designation L-35 was used. According to the CRC L-35 test method, the test bearings are packed with 3.5 cc (or equivalent weight) of grease. Because of the extremely short life of bearings packed with 3.5 cc of grease, the present evaluations were made by packing the bearings completely full with about 6 to 8 grams of grease and using either a standard end cap with no additional grease or a special end cap holding a reservoir of about 10 grams of additional grease. In some tests in the "High Speed Testers" which normally employ only 3.5

cc. of grease, the cavities inside the shields are packed with 4.5 grams of additional grease. The bearing assembly containing an eight-ball SAE No. 204 ball bearing is mounted on a horizontal spindle and in all tests except in the "High Speed Testers" is subjected to a radial load of 5 pounds. In the "High Speed Testers," a radial load of 16 pounds is employed. The portion of the spindle upon which the test bearing assembly is located is encased in a thermostatically controlled oven. By this means the temperature of the bearing can be maintained at a desired elevated temperature. The spindle is driven by a constant belt-tension motor drive assembly, capable of giving spindle speeds up to 45,000 revolutions per minute. The spindle is operated on a cycling schedule consisting of a series of periods, each period consisting of 20 hours running time and 4 hours shutdown time. The test continues until the lubricant fails. The lubricant is considered to have failed when any one of the following conditions occurs, (1) spindle input power increases to a value approximately 300 per cent above the steady state condition at the test temperature; (2) an increase in temperature at the test bearing of 20° F. over the test temperature during any portion of a cycle; or (3) the test bearing locks or the drive belt slips at the start or during the test cycle.

The lubricating oil used in preparing the lubricating composition shown in Table I was a synthetic oil known as QF-6-7024 Fluid marketed by Dow-Corning Corporation. This fluid is considered to be a methyl-phenylsiloxane polymer wherein the "end" silicon atoms are substituted to a high degree by two phenyl groups and one methyl group. The material is highly resistant to radiation. QF-6-7024 Fluid has as typical characteristics a viscosity at 100° F. of about 930 to 1030 SUS, a viscosity at 210° F. of about 90 to 100 SUS, a viscosity index of about 108 to 110 and a pour point of +10° to +20° F.

In preparing the lubricating composition, the oil and the ammeline were mixed at room temperature for a period of 10 to 30 minutes. The slurry thus formed was passed twice through a Premier Colloid Mill set at a stator-rotor clearance of 0.002 inch. The thickened lubricating composition thus prepared had the following approximate make-up and properties.

Table I

|                                     |      |
|-------------------------------------|------|
| Composition, percent by weight:     | A    |
| Lubricating Oil, QF-6-7024          | 65   |
| Amelmine                            | 35   |
| Inspection:                         |      |
| Penetration (ASTM D217-52T):        |      |
| Unworked                            | 306  |
| Worked                              | 306  |
| Dropping point, ° F. (ASTM D566-42) | 900+ |
| Performance life, hrs.:             |      |
| 10,000 r.p.m. at 600° F.            | 93   |
| 20,000 r.p.m. at 400° F.            | 719+ |
| 20,000 r.p.m. at 500° F.            | 455  |
| 20,000 r.p.m. at 600° F.            | 102  |
| 20,000 r.p.m. at 700° F.            | 49   |

The long performance life of the composition of the invention at high rotational speeds and high temperatures is self evident from the above data.

In order to illustrate further the improved lubricating characteristics of a grease composition of the invention, a composition (Composition B) similar to Composition A was prepared employing a synthetic oil known as QF-6-7039 Fluid. QF-6-7039 Fluid is marketed by Dow-Corning Corporation and is believed to be a methylphenylsiloxane polymer inhibited against deterioration and otherwise similar to QF-6-7024. The thickened lubricating compositions using QF-6-7039 had the following approximate make-up and properties.

Table II

|             |                                     |       |
|-------------|-------------------------------------|-------|
| 15          | Composition, percent by weight:     | B     |
|             | Lubricating oil, QF-6-7039          | 65    |
|             | Amelmine                            | 35    |
| Inspection: |                                     |       |
| 20          | Penetration (ASTM D217-52T):        |       |
|             | Unworked                            | 272   |
|             | Worked                              | 275   |
|             | Dropping point, ° F. (ASTM D566-42) | 830+  |
| 25          | Performance life, hrs.:             |       |
|             | 10,000 r.p.m. at 600° F.            | 74    |
|             | 20,000 r.p.m. at 400° F.            | 298   |
|             | 20,000 r.p.m. at 600° F.            | 155   |
|             | 30,000 r.p.m. at 400° F.            | 1509+ |
| 30          | 45,000 r.p.m. at 400° F.            | 149   |

<sup>1</sup> High speed tester.

The long performance life of the composition of the invention (Composition B) at high rotational speeds and high temperatures is readily apparent from an inspection of the data in Table II.

The make-up and properties of other lubricating compositions within the scope of the invention are illustrated in Table III. The DC 550 Fluid used in Compositions C, D and E is marketed by Dow-Corning Corporation and is a methylphenylsiloxane polymer having as typical characteristics a viscosity at 100° F. of 300 to 400 SUS, a viscosity-temperature coefficient of 0.75, a freezing point of -54° F., a flash point of 600° F. and a specific gravity 25° C./25° C. of 1.08. The bis(phenoxy-phenoxy) benzene used in Composition I consists of a mixture of isomers thereof having as typical characteristics a viscosity at 100° F. of about 1691 SUS, a viscosity at 210° F. of about 70.8 SUS and a pour point of +40° F. The m-bis (m-phenoxyphenoxy)phenyl ether used in Compositions J, K and L has as typical characteristics a viscosity at 100° F. of about 8565 SUS, a viscosity at 210° F. of about 118 SUS and a pour point of +70° F. Compositions C to O were subjected to a test using Pope spindles and an MRC 204S-17 bearing at 600° F. and 20,000 revolutions per minute. In these tests the bearings were packed with 7 to 8 grams of grease. A special end cap holding about 10 grams of additional grease was also employed.

Table III

| Composition, Percent By Weight                   | C    | D    | E    | F    | G    | H    | I     | J    | K    | L    | M    | N    | O    |
|--------------------------------------------------|------|------|------|------|------|------|-------|------|------|------|------|------|------|
| Lubricating Oil:                                 |      |      |      |      |      |      |       |      |      |      |      |      |      |
| DC 550 Fluid                                     | 60   | 65   | 32.5 |      |      |      |       |      |      |      | 65   | 65   |      |
| QF-6-7024                                        |      |      | 32.5 | 60   | 72   | 80   | 48.75 |      |      |      |      |      | 70   |
| QF-6-7039                                        |      |      |      |      |      |      | 16.25 |      |      |      |      |      |      |
| Bis(phenoxyphenoxy)benzene                       |      |      |      |      |      |      |       | 72   | 65   | 60   |      |      |      |
| m-Bis(m-phenoxyphenoxy)phenyl ether              |      |      |      |      |      |      |       |      |      |      |      |      |      |
| 1,3,5-Triazine Compound:                         |      |      |      |      |      |      |       |      |      |      |      |      |      |
| Ammelaine (2,4-diamino-6-hydroxy-1,3,5-triazine) | 40   | 35   | 35   | 40   | 28   | 20   | 35    | 28   | 35   | 40   | 35   | 17.5 | 30   |
| Ammelide (2,4-dihydroxy-6-amino-1,3,5-triazine)  |      |      |      |      |      |      |       |      |      |      |      |      |      |
| Inspection:                                      |      |      |      |      |      |      |       |      |      |      |      |      |      |
| Penetration (ASTM D217-52T):                     | 309  | 351  | 324  | 272  | 335  | 392  | 291   | 355  | 328  | 287  | 362  | 335  | 351  |
| Unworked                                         |      |      |      | 343  | 366  | 295  | 265   | 332  | 381  | 275  | 343  | 317  | 321  |
| Worked                                           |      |      |      |      |      | 900+ | 900+  | 900+ | 900+ | 900+ | 900+ | 900+ | 339  |
| Dropping Point, ° F. (ASTM D566-42)              | 900+ | 800+ | 900+ | 900+ | 900+ | 900+ | 900+  | 900+ | 900+ | 900+ | 900+ | 900+ | 850+ |
| Performance Life, hrs., 20,000 r.p.m. at 600° F. | 85   | 91   | 97   | 81   | 103  | 79   | 76    | 70   | 96   | 78   | 117  | 105  | 77   |

The long performance life of compositions of the invention is readily apparent from an inspection of the data in Table III.

Other lubricating compositions within the scope of the invention are illustrated in Table IV.

wherein  $R_1$  is selected from the group consisting of hydrogen, alkyl, aryl, alkaryl, aralkyl, cyanoalkyl, pyridyl, hydroxy and mercapto radicals.

6. The lubricating composition of claim 5 wherein the 5 lubricating oil is a polyorgano siloxane.

Table IV

| Composition, Percent By Weight                       | P  | Q  | R  | S  | T  | U  | V  | W  | X  | Y  | Z  | A' | B' | C' | D' |
|------------------------------------------------------|----|----|----|----|----|----|----|----|----|----|----|----|----|----|----|
| Lubricating Oil:                                     |    |    |    |    |    |    |    |    |    |    |    |    |    |    |    |
| DC 550 Fluid                                         | 60 | 65 | 70 | 75 | 80 | 60 | 65 | 70 | 75 | 80 | 60 | 65 | 70 | 75 | 80 |
| QF-6-7024                                            |    |    |    |    |    |    |    |    |    |    |    |    |    |    |    |
| Di-2-ethylhexyl sebacate                             |    |    |    |    |    |    |    |    |    |    |    |    |    |    |    |
| 1,3,5-Triazine Compound:                             |    |    |    |    |    |    |    |    |    |    |    |    |    |    |    |
| Benzoguanamine (2,4-diamino-6-phenyl-1,3,5-triazine) | 40 |    |    |    |    |    |    |    |    |    |    |    |    |    |    |
| Ammelide (2,4-dihydroxy-6-amino-1,3,5-triazine)      |    | 35 |    |    |    |    |    |    |    |    |    |    |    |    |    |
| Ammeline (2,4-diamino-6-hydroxy-1,3,5-triazine)      |    |    | 30 | 25 |    | 20 | 40 | 35 | 30 | 25 |    |    |    |    |    |
| 2,4-Dihydroxy-6-pyridyl-1,3,5-triazine               |    |    |    |    |    |    |    |    |    |    |    |    |    |    |    |
| 2,4-Dimercapto-6-amino-1,3,5-triazine                |    |    |    |    |    |    |    |    |    |    |    |    |    |    |    |
| 2,4-Diamino-1,3,5-triazine                           |    |    |    |    |    |    |    |    |    |    |    |    |    |    |    |
| 2,4-Diamino-6-methyl-1,3,5-triazine                  |    |    |    |    |    |    |    |    |    |    |    |    |    |    |    |
| 2,4-Diamino-6-ethyl-1,3,5-triazine                   |    |    |    |    |    |    |    |    |    |    |    |    |    |    |    |
| 2,4-Diamino-6-n-butyl-1,3,5-triazine                 |    |    |    |    |    |    |    |    |    |    |    |    |    |    |    |
| 2,4-Diamino-6-benzyl-1,3,5-triazine                  |    |    |    |    |    |    |    |    |    |    |    |    |    |    |    |
| 2,4-Diamino-6-p-tolyl-1,3,5-triazine                 |    |    |    |    |    |    |    |    |    |    |    |    |    |    |    |
| 2,4-Diamino-6-naphthyl-1,3,5-triazine                |    |    |    |    |    |    |    |    |    |    |    |    |    |    |    |
| 2,4-Diamino-6-cyanoethyl-1,3,5-triazine              |    |    |    |    |    |    |    |    |    |    |    |    |    |    |    |
| 2,4-Diamino-6-cyanobutyl-1,3,5-triazine              |    |    |    |    |    |    |    |    |    |    |    |    |    |    |    |
| 2,4-Diamino-6-cyanoctyl-1,3,5-triazine               |    |    |    |    |    |    |    |    |    |    |    |    |    |    |    |
| 2,4-Diamino-6-cyanoctyl-1,3,5-triazine               |    |    |    |    |    |    |    |    |    |    |    |    |    |    | 20 |

While our invention has been described with reference to various specific examples and embodiments it will be understood that the invention is not limited to such examples and embodiments and may be variously practiced within the scope of the claims hereinafter made.

We claim:

1. A lubricating composition capable of functioning at temperatures up to about 600° F. consisting of a dispersion in a lubricating oil selected from the group consisting of polyorgano siloxanes, organic esters and polyaryl ethers of a sufficient amount to thicken the lubricating oil to a grease consistency of a 1,3,5-triazine compound melting above about 205° C. having the following 40 formula:



wherein R and  $R_1$  are selected from the group consisting of hydrogen, alkyl, aryl, alkaryl, aralkyl, cyanoalkyl, pyridyl, amino, hydroxy and mercapto radicals, R and  $R_1$  being unlike radicals when selected from the group consisting of amino, hydroxy and mercapto radicals.

2. The lubricating composition of claim 1 wherein the 45 1,3,5-triazine compound comprises about 20 to about percent by weight of the total composition.

3. The lubricating composition of claim 1 wherein the lubricating oil is a polyorgano siloxane.

4. The lubricating composition of claim 1 wherein the lubricating oil is a polyphenyl ether.

5. A lubricating composition capable of functioning at 65 temperatures up to about 600° F. consisting of a dispersion in a lubricating oil selected from the group consisting of polyorgano siloxanes, organic esters and polyaryl ethers of a sufficient amount to thicken the lubricating oil to a grease consistency of a guanamine derivative melting above about 205° C. having the following formula:



7. The lubricating composition of claim 5 wherein the lubricating oil is a polyphenyl ether.

8. A lubricating composition capable of functioning at temperatures up to about 600° F. consisting of a dispersion in a liquid polyorgano siloxane of a sufficient amount to thicken the polyorgano siloxane to a grease consistency of ammeline.

9. A lubricating composition capable of functioning at temperatures up to about 600° F. consisting of a dispersion in a liquid polyorgano siloxane of a sufficient amount to thicken the polyorgano siloxane to a grease consistency of ammelide.

10. A lubricating composition capable of functioning at temperatures up to about 600° F. consisting of a dispersion in a liquid polyphenyl ether of a sufficient amount to thicken the polyphenyl ether to a grease consistency of ammeline.

11. A lubricating composition capable of functioning at temperatures up to about 600° F. consisting of a dispersion in a liquid polyphenyl ether of a sufficient amount to thicken the polyphenyl ether to a grease consistency of ammelide.

12. A lubricating composition capable of functioning at temperatures up to about 600° F. consisting of a dispersion in a liquid polyorgano siloxane of a sufficient amount to thicken the polyorgano siloxane to a grease consistency of a mixture of ammeline and ammelide wherein the weight ratio of ammeline to ammelide is about 1:1.

References Cited in the file of this patent

UNITED STATES PATENTS

2,984,624 Halter et al. May 16, 1961